

## UNITED STATES PATENT OFFICE.

FRANCIS G. OKIE, OF PHILADELPHIA, PENNSYLVANIA, ASSIGNOR TO MINNESOTA MINING & MANUFACTURING COMPANY, OF ST. PAUL, MINNESOTA, A CORPORATION OF MINNESOTA.

## COMPOSITE ADHESIVE AND PROCESS OF MAKING SAME.

No Drawing.

Application filed March 4, 1922. Serial No. 541,249.

My present invention relates in general to the treatment of material, preferably in sheet form, and more particularly the treatment of material for the purpose of forming or attaining composite structures, of which well known forms of abrasives such as what is commonly known as sand-paper is an example.

This application is a continuation in part 10 of my applications, Serial Number 428,287 and 428,289.

Although I hereinafter disclose the practice of my invention in connection with abrasives such as sand-paper, it will be understood 15 that my invention, or certain features thereof, have a wider field of utility.

Composite structures of the abrasive type such as sand-paper or emery cloth comprise generally (a) a backing of sheet material, 20 which may be felted as in the case of paper or woven as in the case of cloth, (b) a more or less finely comminuted resistant material having abrading properties, such as garnet or corundum, and (c) a binder generally in 25 the form of a glue which serves to bind the abrasive to the backing.

The binders as produced at present have as incidents certain features among which are (1) defect of desired drying qualities, 30 (2) affinity for moisture rendering them substantially inutile in the presence of water or moisture, (3) the tendency to premature pulverization or disintegration of the binder when exposed to normal atmospheric conditions and other undesired drying qualities, 35 and (6) cracking, with consequent exposure of the base, when bent.

The principal objects of my present invention are the provision of a binder which 40 functions more efficiently than any known to me; the provision of a binder characterized by flexibility without cracking or other undesirable effects; the provision of a binder characterized by extensibility and compressibility to accommodate itself to flexion 45 of the backing; the provision of a binder by means of which the desired adhesive action between it and the backing is attained not only efficiently but also with a desirable 50 degree of acceleration, and more particularly the provision of a binder in which the drying action will be effective from the contact surface between it and the backing outwardly; the provision of a binder in which

the drying action will be effective from the 55 outer surface thereof inwardly; the provision of a binder characterized by a drying action that permits of handling the product with a minimum of delay and more particularly such handling without impairment of 60 the superficies of the material; the provision of a binder characterized by an accelerated drying action; the provision of a binder the rate of speed of whose drying is subject to variation; and the provision of a 65 binder having moisture-proofing functions.

In the employment of my present invention for the production of sand-paper and the like (which I cite for purposes of example) I use as the backing a sheet of material (which may be paper) as will conveniently serve the employment contemplated, and as the abrasive such comminuted material (which may be crushed garnet) similarly adapted to serve the function in view. 70

It is desirable that the binder utilized have the functions and characteristics not only of great mechanical strength and of great binding strength, but also that it be non-hygroscopic, permeative, moisture resistant, easily worked, readily obtainable, inexpensive and facilely applied. 80

I have discovered that resins including some which are commonly called gums of such types as are used in the manufacture of 85 the better grades of varnish are peculiarly adapted for the attainment of these ends and that resins such as kauri, copal, dammar are examples of these types. Gum dammar is preferred by me as best attaining the desired ends, viewed from certain aspects.

In preparing the binder for use, the resin is used in connection with a suitable vehicle which I prefer is of a type such as linseed oil or China wood oil, for reason which I 95 will proceed to explain.

In applying a resin prepared with a vehicle such as linseed oil to one surface of a backing of paper for example I have found that the action of the vehicle involves 100 a penetration of the backing by the vehicle, for example linseed oil, to a point which approximates the opposite surface of the sheet but falls short of actual exudation of the vehicle upon such opposite surface thereby preventing starving of the joint between the abrasive and the adhesive or backing or both.

This results in a moisture-proofing of the material even against the absorption of moisture through the surface opposite to that to which the binder is applied, without at the same time defacing or otherwise undesirably affecting such opposite surface.

- This penetration by the vehicle, particularly when coupled with the use of the character of resin pointed out above, carries with it in such penetration a certain amount of finely divided resin so that a coating and binding action is secured between the fibres or elemental portions of the backing which thus substantially retards, if it does not entirely prevent, disintegration of the backing, in addition to preventing access of moisture through the backing to the plane of contact between the backing and the main mass of the binder material.
- The efficient action of the binder may be enhanced in the manufacture of sand-paper if the binder is applied to the backing by the use of pressure and the more or less finely divided abrasive is then applied in such a manner as to cause it to adhere to the binder.

In order to accelerate the adhesion between the binder and the backing, I have discovered it desirable to use with the binder a modifying agent the action of which is to cause a siccative and/or hardening of the binder initiated at the contact surface of the binder with the backing and effective outwardly.

In my experience I have discovered that there are a number of metallic compounds which are useful for my present purposes, that manganic oxides are peculiarly useful and that borate of manganese best combines siccative and hardening properties with the desirable and susceptibility to fine grinding.

Due to the relatively slow drying of binders generally, difficulties are encountered in handling the abrasive structure, within a convenient period because of the soft and sticky character particularly of the exposed surfaces of the binder. This objection I mitigate by associating with the improved binder a substance the action of which is to produce an accelerated drying action effective primarily at the exposed surface and working inwardly, and for this purpose I incorporate in the binder a modifying element peculiarly effective in its action as an oxidizing agent on such vehicles as linseed oil and as a retarding agent with reference to the excess absorption of the vehicle by the backing.

The substance I have discovered to be particularly adapted for this purpose is carbonate of lead or white lead which is a new electrolytic process white lead and which in my experience is found to be more satisfactory than any other known form of carbonate of lead.

Whereas by itself the aforementioned

white lead adds but relatively little strength to the binder, in association in the binder with the borate of manganese it intensifies the action of the binder in holding the abrasive firmly against the backing.

For increasing the adhesive properties of the binder, and for hastening the drying thereof, I have discovered that it is desirable to employ a paste dryer (so-called because it is formed in the nature of a paste) which is also efficacious in holding the mineral particles such as grit in suspension in the binder without loss of siccative properties and without appreciably reducing the desired fluidity of the binder. This may comprise such metallic compounds as sugar of lead and borate of manganese suspended in a suitable vehicle such, for instance, as linseed oil or linseed oil with a resin, but I find it preferable to form the paste dryer so as to have the metallic compounds contained therein in the form of acetate of lead and resinate of manganese. I have found by experience that the paste dryer should be somewhat in the nature of cheesy butter, rather softer, and of a light brownish grey color.

As an auxiliary in (1) accentuating the adhesion of the binder to the paper, (2) facilitating to a certain extent the spreading of the binder, and (3) modifying as desired the consistency of the binder as is useful in cases where it is desired to render it more fluid, I have discovered that the use of a japan dryer is desirable. Such a dryer which is relatively free from rosin is to be preferred. One form of this contains shellac, red lead, litharge, manganese oxid, burnt umber, resin, linseed oil, and turpentine quantum sufficit.

In order to give the binder the desired fluidity, viscosity and bulk I preferably employ a varnish consisting largely of linseed oil boiled until it reaches nearly a solid state. As far as practicable and feasible uncombined fatty acids and glycerin should be eliminated. I have employed a linseed oil successfully for this purpose having an iodine number as low as 185, but prefer that of having an iodine number as high as 190.

The aforementioned resins, such as gum dammar are preferably employed in the form of a varnish which is substantially three parts Batavia dammar, steam kettle melted, with two parts kettle boiled linseed oil.

While gum copal and gum kauri in certain respects make more substantial binders than gum dammar, as they will carry more oil and dry harder under certain conditions as may be useful for certain purposes, generally speaking the present relatively greater expense does not ordinarily justify their use for most purposes, which are well served by gum dammar.

Though I have hereinabove disclosed cer-

tain forms of useful dryers having various characteristics, and likewise, I have discovered that where it is advisable that the sic-  
cative action thereof be limited, or at least retarded, that it is desirable to incorporate in the binder a non-drying oil such as castor oil or the like, for such purposes.

Sand-paper made in accordance with the disclosure of my present invention is characterized by great flexibility without any adverse effects, such as cracking of the binder or backing, or loosening of one from the other.

In my preferred practice, as will hereafter appear, I form batches which by weight and percentage contain the following ingredients:

|          |                     | Lbs.     |
|----------|---------------------|----------|
| Part I   | Carbonate of lead   | 24 .1666 |
| 20       | Gum varnish         | 6 .0416  |
| Part II  | Borate of manganese | 6 .0416  |
|          | Gum varnish         | 6 .0416  |
| Part III | Japan dryer         | 6 .0416  |
| 25       | Paste dryer         | 6 .0416  |
|          | Linseed oil varnish | 48 .3333 |
|          | Gum varnish         | 42 .2916 |

In such preferred practice, Parts I and II are mixed and milled separately since Part I mills more readily than Part II, and are desirably then mixed with Part III and the composite batch is then milled until smooth.

Parts I and II include the gum varnish in order to attain not only a fine subdivision of the metallic substance but also to render them readily miscible with Part III.

The materials used by me as hereinabove described may be varied in character so as to vary the characteristics of the binder from the stand-point of adhesiveness, non-hygroscopy, and flexibility. Where such variation in the use of materials is employed to produce, for instance, increased adhesion between the binder and the abrasive, such increase may be attained though possibly at a certain expense in its characteristic of flexibility.

By this process I am enabled to obtain sand-paper characterized by extraordinary thinness and flexibility, in that I am able to form sand-paper and the like with a backing so thin that such product could not be manufactured, if the backing originally used were of the thinness ultimately desired.

In the preferred practice of my invention, in forming Part I hereinabove referred to, I grind the carbonate of lead and the gum varnish to an exceeding fineness which may be accomplished by passing them through a fine-grinding mill three or four trips. The material grinds quickly and easily and may be conveniently mixed in the mill. One of the functions of the carbonate of lead is to hasten the oxidization of the thinner (and

greasier) elements of the binder and limit their absorption by the backing, e. g., paper in the case of sand-paper. It also hastens the superficial top-drying of the sand-paper or the like, rendering it among other things easier to handle before it becomes dry. Ordinary white leads, even though of apparent equal purity and of similar analyses as that herein referred to, do not function as satisfactorily for chemical reasons not yet brought to light by my experience.

Gum varnish may be No. 1 gum kauri, gum copal, or gum dammar or more or less numerous similar suitable resins commonly called gums melted in boiled or raw linseed oil, with or without the presence of dryers, such as red lead, litharge, black oxid of manganese, burnt umber, and the like. The gum varnish preferably used by me in Parts I, II and III above referred to, is substantially equal parts Batavia dammar gum, steam kettle melted, and kettle boiled linseed oil. While I preferably use gum dammar, as just indicated, I have formed a gum dammar varnish made from three parts Batavia dammar, melted by itself under gentle heat, as is preferable though it may be used cold, and two parts of a hydrocarbon (which may be one of the petroleum series)—obviously added after the heat, if used, is discontinued. The hydrocarbon referred to preferably takes the following form:—Color, water white; Beaumé, 48°-49°; initial boiling point, not below 275° F.; not more than 50% over, at 340° F.; recovery, at least 95%; residue, colorless; end point, below 475° F.

As the hydrocarbon evaporates, it may be advisable to add more to the mixture in order to preserve the desired degree of fluidity. The hydrocarbon dammar varnish thus formed makes a more brittle binder than the linseed oil gum dammar varnish above described. Although gum copal and gum kauri each make a more substantial binder than gum dammar, as they carry more oil and dry harder, they are more expensive. Gum dammar, though not oxidizing to such a degree of hardness and toughness as other gums mentioned, is preferable for my purpose because it approximates as nearly as possible the desirable properties of kauri, but approaches in cost rosin without including all the undesirable characteristics thereof and goes as far in the direction of the employment of common rosin as I am at present advised is safe to do.

I have found that synthetic resins can also be used in place of natural resins, sometimes called gums, to good advantage in making a binder for my purposes. An example of such a synthetic resin is that known to the trade as bakelite resin, or commercial phenol resin produced by a condensation process.

In using borate of manganese I have found

that a well known borate of manganese, readily obtainable in the open market combines best siccative properties with susceptibility to fine grinding and to form Part II referred to above it should be ground in the varnish until it may be spread on a glass without being mealy under one's finger. It should be ground until experience shows that it can be ground no finer.

10 It will be understood from the foregoing reference to drying intensifiers that the siccative properties of the borate of manganese constituent are such as to include facilitating drying outwardly of the binder from the 15 surface in contact with the backing, and that the carbonate of lead constituent includes causing drying inwardly of the binder from the surface thereof which is in contact with the air.

20 While I prefer to employ manganese compounds in the form of borate of manganese, it is to be observed that although black oxide of manganese contains certain desirable siccative elements for my purposes, it does not 25 readily lend itself to grinding in such a manner as is desired by me. At times, advantage may be taken of the characteristics of black oxide of manganese as a drier by heating it in linseed oil and using this mixture.

30 Similarly, cobalt derivatives, (such as acetate of cobalt) may be employed for their siccative qualities, but I have found that due care should be employed in using such highly concentrated dryers so as to avoid any 35 tendency toward deterioration and relative inactivity with the other dryers; failing such care such cobalt derivatives do not give such excellent effects as borate of manganese.

In forming Part II according to my preferred practice, I find it desirable to grind the borate of manganese by itself, ten or 40 twelve trips if necessary, as this is relatively a very hard substance to grind, and the varnish may be mixed therewith in the mill.

45 The form of japan-dryer preferably employed by me is a well-known japan which contains about 2% (two percentum) of shellac, preferably the best obtainable, besides substances such as red lead ( $Pb_3O_4$ ) litharge 50 ( $PbO$ ) manganese-oxid ( $MnO$ ) burnt umber (which has a manganese and oxygen content) and resins in linseed oil and turpentine. It aids in the binding action and acts to some extent as a thinner whose turpentine content evaporates after the binder is 55 spread on the paper and somewhat facilitates the spreading process. I have the proportion of japan dryer indicated in Part III as ordinarily adequate but yet capable of increase with safety when larger quantities 60 are desirable. Although to an unaccustomed observer a rosin content in the japan may, due to its rapidity of action, appear to be advantageous, such a content is within my 65 experience undesirable, and to be avoided.

To form the linseed oil varnish of Part III herein referred to, I prefer to employ a linseed oil as free as possible from uncombined fatty acids and glycerin, reached by boiling a high grade linseed oil until nearly 70 solid. While this is more difficult to handle, I find that it possesses to a high degree the ideal balance between fatty acids and glycerides, so that it neither overoxidizes nor does it dry sticky.

75 In preparing the paste-dryer of Part III above referred to, which preferably incorporates two separately prepared compositions, I first form the initial portion of the dryer by stirring 200 pounds of litharge ( $PbO$ ) and 200 pounds of hot water ( $120^{\circ} F.$ ), the agitation of the water being sufficiently violent during and after the addition of the litharge to keep it from settling. After, say, two to five minutes of this sustained agitation, 45 pounds of 80% acetic acid is dashed into the hot-water and litharge composition without cessation of the violent stirring, which may be mechanical agitation, and which should continue until the milky white liquid that develops as soon as the acid strikes the water and litharge, sets to a consistency resembling soft cottage cheese or bonny clabber and offers resistance enough to tend to slow up a strong man using a 90 paddle.

95 In cases where a mechanical agitator is used, it should be shut off at this stage which is ordinarily reached within a minute after the acetic acid is dashed in. It is advisable to have the agitation sufficiently violent to cause suspension of all of the litharge and to dash in the acetic acid suddenly, as otherwise a quantity of uncombined litharge will 100 be found at the bottom of the mixer, and the mass, which is now basic acetate of lead, will not set stiff. This resultant mass should be undisturbed for about 15 hours and then 75 pounds kettle boiled linseed oil is added to the mass, which by this time has become somewhat stiffer. The whole mass is then 105 mixed preferably in a mechanical mixer. The mixer should be run until a large percentage of the original water may be poured off. At this time the basic acetate of lead has a greater affinity for the oil than for the water. When further agitation separates out no more water, the compound should be ground. This may be done on 3 roller ink mill until no more water can be discerned, and when substantially all of it can be accounted for by weighing the water that has 115 been poured off. The strength of the acetic acid may be varied below 80% provided the proportions are changed correspondingly to the strength of the acetic acid. This forms the first part or composition of the paste 120 dryer.

125 While the second part of the paste dryer may be heated during formation, I prefer to 130

mix thoroughly 100 pounds of kettle boiled linseed oil, with 75 pounds of resinate of manganese (powdered form) and then grind the mixture two or three trips until fine and 5 smooth.

I then add 225 pounds kettle boiled linseed oil to the acetic acid treated litharge formed in the mixer as above set forth, and then quickly mix the resulting mass of the 10 second resinate manganese composition with the modified first or lead compound portion which is in the mixer as just set forth.

In further explanation of the above it is pointed out that I provide a mixture A, 15 that is the first part or composition of the paste drier which is a reaction product of litharge and acetic acid; then the second part B is made which is linseed oil, treated by resinate of manganese; then certain modification of the portion A is afforded to get 20 AC; namely, adding linseed oil to the part A. When this is accomplished I add AC to B and thus obtain the complete mixture D.

This mixing of the two portions should 25 be done quickly because there is a nicely balanced proportion between the two, and an excess of either portion in long contact with the other portion, imperfectly mixed, causes a livering and sometimes a separation there- 30 between. After this mixture of the two portions has stood for substantially an hour, they should be milled one trip. This completes the paste drier. It should flow down the apron of the mill about one inch deep, 35 (more or less, depending partly on tightness of rollers and consequent heat,) and it should be kept in stock in a consistency about like cheesy butter, but rather softer, and of a light brownish gray color.

40 The manganese compound may be made from a resin other than rosin which for my purpose may be dammar, kauri or similar compounds which in the paste drier will in the final product render the same more te- 45 nacious, stable and of augmented physical properties.

From the foregoing description it will be apparent that one of the general functions of the carbonate of lead is to serve primarily 50 as a filler; and of the borate of manganese, as well as of the japan composition referred to, is to serve primarily as a dryer, and that the rest of my improved binder is made up of varnishes.

The gross formula of the binder produced 55 by my method considered from this just re-cited aspect of the invention, therefore in- 60 volves the use, generally, of four parts "filler", three parts "dryer", and seventeen parts "varnish", preferably associated to- 65 gether in the specific manner set forth.

The binder is formed, in my preferred 70 practice, by running together through the mill Parts I and II, ground finely as de- 66 scribed, together with the items of Part III,

all three parts being milled together until the whole mass is uniform and smooth. The binder thus formed should be kept carefully covered preferably in contact with oiled paper to prevent the formation of surface skin 70 through exposure.

Having thus described my invention and illustrated its use, what I claim as new and desire to secure by Letters Patent is—

1. The process of producing a binder for 75 sandpaper which includes admixing lead carbonate as an oxidizing agent with a varnish, combining the same with a varnish including a compound of manganese as a sic- 80 cative and adding a drying oil and a drier thereto, whereby the whole is adapted to harden or congeal into a substantially stable, flexible form or condition for forming a coating which will adhere both to the sup- 85 porting backing and abrasive particles. 85

2. The process of producing a binder for sandpaper which includes admixing a com- 90 pound of a heavy metal as an oxidizing agent with varnish, combining the same with a varnish including a compound of manga- 95 nese, adding a drier and linseed oil varnish, whereby the whole is adapted to harden or congeal into a substantially stable, flexible form or condition for forming a coating which will adhere both to the supporting 95 backing and abrasive particles.

3. The process of producing a binder for 100 sandpaper which includes admixing a com- 105 pound of a heavy metal as an oxidizing agent with a gum varnish, combining the same with linseed oil including a drier and adding a varnish including linseed oil, a resinate of manganese and basic acetate of lead, whereby the whole is adapted to harden or congeal into a substantially stable, flexible 110 form or condition for forming a coating which will adhere both to the supporting 115 backing and abrasive particles. 105

4. The process of producing a binder for 110 sandpaper which includes admixing lead carbonate with a gum varnish, combining the same with a gum varnish including a sic- 115 cative and with linseed oil varnish together with the reaction product of basic lead acetate and resinate of manganese whereby the 120 whole is adapted to harden or congeal into a substantially stable, flexible form or condition for forming a coating which will adhere both to the supporting backing and abrasive particles. 120

5. The process of producing a binder for sandpaper which includes preliminarily forming individual batches of varnish each including, respectively, a compound of a heavy metal as an oxidizing agent, a sicca- 125 tive, and a paste drier comprising the re- 125 action product of basic lead acetate and manganese resinate, combining said batches whereby the whole is adapted to harden or congeal into a substantially stable, flexible 130

form or condition for forming a coating which will adhere both to the supporting backing and abrasive particles.

6. The process of producing a binder for sandpaper which includes preliminarily forming individual batches of varnish, each of said batches including, respectively, a filler having oxidizing properties and a siccative, combining said batches, then adding a linseed oil varnish whereby the whole is adapted to harden or congeal in a substantially stable or flexible form or condition for forming a coating which will adhere both to the supporting backing and abrasive particles.

7. In the process of preparing a binder for sandpaper including a gum varnish, the step which includes preparing a basic acetate of lead in an aqueous medium and separating the basic acetate of lead from the medium in which it is formed by the addition thereto of a vehicle soluble in the varnish.

8. The process of producing a binder for sandpaper which includes admixing lead carbonate with a varnish therefor combining the same with a varnish material including borate of manganese, adding a paste drier including the reaction product of basic acetate of lead and a resinate in linseed oil whereby a composition is obtained adapted to form a substantially stable, flexible coating which will adhere both to the supporting backing and abrasive particles.

9. The process of making a binder including metallic compounds serving as a filler and an oxidizer, gum varnish, linseed oil varnish and a drier which includes the steps

of preparing individual batches of said compounds and gum varnish and of said oxidizer and gum varnish and combining therewith an additional quantity of gum varnish, linseed oil varnish and a paste drier, whereby the whole is adapted to harden or congeal into a substantially stable, flexible form or condition for forming a coating which will adhere both to the supporting backing and abrasive particles.

10. The process of producing a binder for sandpaper which includes combining with a gum varnish, a mixture comprising a powdered, body augmenting agent in a vehicle soluble in the varnish and including a gum, adding a drier thereto and an additional quantity of gum varnish, whereby the whole is adapted to harden or congeal into a substantially stable, flexible form or condition for forming a coating which will adhere both to the supporting backing and abrasive particles.

11. The process of producing a binder for sandpaper which includes combining with an oil varnish, a mixture comprising a normally dry, powdered body augmenting agent in a vehicle soluble in said varnish, adding a drier thereto and an additional quantity of a drying oil varnish whereby the whole is adapted to harden or congeal in a substantially stable, flexible form or condition for forming a coating which will adhere both to the supporting backing and abrasive particles.

In testimony whereof I have hereunto signed my name.

FRANCIS G. OKIE.